

# United States Patent Office

3,695,885

Patented Oct. 3, 1972

1

3,695,885

## HEAT DEVELOPABLE DIAZOTYPE COPYING MATERIAL

Shoji Maryama, 4100 Isobe, Sagamihara-shi, Japan; Tadashi Saito, 30 Kitamigata, Kawasaki-shi, Japan; and Tomiaki Asami, 280 Hiyoshi-cho, Kohoku-ku, Yokohama-shi, Japan

No Drawing. Filed June 5, 1970, Ser. No. 43,968  
Claims priority, application Japan, June 7, 1969,  
44/17,475; Feb. 28, 1970, 45/44,745

10 Int. Cl. G03c 1/54, 1/58, 1/60 27 Claims

### ABSTRACT OF THE DISCLOSURE

A heat developable diazotype copying material comprising a support and a light-sensitive layer formed onto one surface of said support, said layer containing a coupler which activated during the heat development of the copying material and at least two kinds of diazonium compounds forming a black azo dye as a result of a reaction between said coupler and said diazonium compounds.

### BACKGROUND OF THE INVENTION

#### (1) Field of the invention

The present invention relates to a diazotype copying material capable of forming a desired black copied-image through heat development.

#### (2) Description of the prior art

The conventional heat developable diazotype copying materials may be divided broadly into three categories as follows by the components of the light-sensitive layer thereof and the pattern of the heat development process applicable thereto.

(a) Copying materials whose light-sensitive layer contains diazonium compounds, a coupler and an alkali-producing agent capable of producing ammonia gas when heated, such as urea, so that the coupling is effected by virtue of alkali produced by heating the copying material at the time of development thereof.

(b) Copying materials whose light-sensitive layer contains an alkali salt of an acid such as trichloroacetic acid which may be decomposed by heating to form an alkali producing agent, so that the coupling is effected by means of alkalizing the light-sensitive layer by heating the copying material at the time of development thereof.

(c) Copying materials whose light-sensitive layer does not contain any alkaline component, but contains a coupler together with diazonium compound, said coupler being activated and combined with said diazonium compounds when heated, so that the coupling is effected by heating the copying material at the time of development thereof.

### SUMMARY OF THE INVENTION

The object of the present invention is to provide a heat developable diazotype copying material of the foregoing category (c), and particularly materials which are capable of effecting the coupling of a copied image in black color tone.

The coupler constituting one component of the light-sensitive layer applicable in the present invention, it includes such compounds as expressed by the following general formula:



2

wherein:

R<sub>I</sub> and R<sub>III</sub> each is a radical selected from the group consisting of hydrogen, alkyl radicals having 1 to 6 carbon atoms, benzyl, bromine, chlorine, iodine, acetyl, and  $\omega$ -carboxyalkyl radicals having 1 to 4 carbon atoms; and R<sub>II</sub> is a radical selected from the group consisting of hydrogen, hydroxyl radical alkyl radical having 1 to 2 carbon atoms, alkyl-sulfonyloxy ( $-\text{O}-\text{SO}_2\text{-alkyl}$ ) radicals in which the alkyl group has 1 to 4 carbon atoms, carboalkoxyoxy



radicals in which the alkyl group has 1 to 4 carbon atoms, acylacyoxy



radicals having 7 to 9 carbon atoms, alkylacyloxy



radicals having 2 to 12 carbon atoms,  $\omega$ -hydroxyalkyl radicals having 1 to 3 carbon atoms,  $\omega$ -hydroxyalkyl oxy radicals having 1 to 3 carbon atoms and alkoxy radicals having 1 to 4 carbon atoms; and

25 R<sub>II</sub> is a radical selected from the group consisting of hydrogen, hydroxyl radical, alkyl radicals having 1 to 2 carbon atoms, alkoxy radicals having 1 to 4 carbon atoms, sulfonyloxy ( $-\text{O}-\text{SO}_2-$ ) radical, alkyl-sulfonyloxy ( $-\text{O}-\text{SO}_2\text{-alkyl}$ ) radical in which the alkyl group has 1 to 4 carbon atoms, carbamoyl radical, carbamoyloxy radical, carboalkoxyloxy radicals in which the alkoxy group has 1 to 4 carbon atoms, acyl oxy radicals in which the acyl group has 2 to 9 carbon atoms, alkyl-acyloxy radicals having 2 to 12 carbon atoms,  $\omega$ -hydroxyalkyl radicals having 1 to 3 carbon atoms and  $\omega$ -hydroxyalkyloxy radicals having 1 to 3 carbon atoms.

30 The foregoing coupler is combined with at least one member selected from the group consisting of diazonium compounds expressed by the below-mentioned general Formulas I and I' and at least one member selected from the group consisting of such diazonium compounds as expressed by the below-mentioned general Formulas II to IV which is capable of coupling in blue color or purple color as a result of a reaction effected between said coupler and the diazonium compound.



wherein:

Y is a member selected from the group consisting of



55 (wherein R' represents a radical selected from the group consisting of hydrogen, alkyl radicals having 1 to 4 carbon atoms, hydroxyethyl radical, hydroxypropyl radical and acetyl radical); and X is a member selected from the group consisting of  $-\text{Cl}\cdot\frac{1}{2}\text{ZnCl}_2$ ,



(II)

wherein:

R'' is a radical selected from the group consisting of hydrogen, cyclohexyl radical, alkyl radicals having 1 to 4 carbon atoms, hydroxyalkyl radicals having 2 to 4 carbon atoms, cyano radical and aralkyl radicals having 7 to 11 carbon atoms, such as



R''' is a radical selected from the group consisting of 10 alkyl radicals having 1 to 4 carbon atoms, aralkyl radicals having 7 to 11 carbon atoms, such as



cyclohexyl radical, hydroxyalkyl radicals having 2 to 4 carbon atoms and benzoyl radical; and X' is the radical identical with that of said X expressed in the general Formula I.

Specific examples of diazonium compounds within the scope of general Formula I, are such compounds as:



Specific examples of diazonium compounds within the scope of general Formula I', are such compounds:



Diazonium compounds of dialkylaniline group expressed by the following general Formula II:



wherein:

R'''' and R''''' each is a radical selected from the group consisting of alkyl radicals having 1 to 4 carbon atoms, hydroxylalkyl radical having 2 to 3 carbon atoms and benzyl radical; and

"X'" is the radical identical with that of X expressed in the general Formula I.

Diazonium compounds expressed by the following general Formula III:



wherein:

$X'''$  and  $Y'$  are the radicals identical with that of  $X$  and  $Y$ , respectively, expressed in the general Formula I; and

and  
 $R_{IV}$  and  $R_V$  each is a radical selected from the group consisting of alkoxyl radicals having 1 to 4 carbon atoms, halogens and hydrogen.

Diazonium compounds of benzoyl amide group expressed by the following general Formula IV:



wherein:

R<sub>VI</sub> and R<sub>VII</sub> each is a radical selected from the group consisting of alkoxyl radicals having 1 to 4 carbon atoms, halogens and hydrogen;

R<sub>VIII</sub> is a radical selected from the group consisting of hydrogen and alkyl radicals having 1 to 3 carbon atoms; and X<sup>''''</sup> is the radical identical with that of X expressed in the general Formula I.

A coupler expressed by the above-mentioned general formula usually forms a purple azo dye or a blue azo dye as a result of a coupling reaction between said coupler and a diazonium compound generally employed for conventional diazotype copying materials, but in case where a coupling reaction is effected between said coupler and a member selected from the group consisting of diazonium compounds expressed by the foregoing general Formulas I and I' along with a member selected from the group consisting of diazonium compounds expressed by the foregoing general Formulas II, III or IV, there is formed a black azo dye. And, in case where a coupling reaction is effected between said coupler and a single member selected from the group consisting of diazonium compounds expressed by said general Formula I or general Formula I', there is formed a yellow azo dye.

In other words, the present invention stems from the knowledge obtained through observation and study of the coupling reaction effected by means of varieties of combinations of diazonium compounds and coupler. At least one member as illustrated by Formulas I and I' must be contained in the light-sensitive layer of the copying material. Diazonium compounds expressed by the general Formulas II through IV represent the optimum examples.

but any other diazonium compound generally employed in this field of art and capable of forming a blue azo dye or a purple azo dye as a result of coupling reaction between a coupler expressed by the foregoing general formula and said diazonium compound is also applicable in the present invention.

In addition to the diazonium compounds and the coupler as mentioned above, an organic acid such as citric acid, tartaric acid, etc. as the acid component contributing to the preservability of the copying material, thiourea contributing to the prevention of fading as well as the preservability of the copying material, and so-called coupling assistant such as guanidine sulfate, pentaerythritol, O-methyl-isothiourea, guanylurea, etc. contributing to accelerating the coupling can be also employed as a component of the light-sensitive layer in the same way as in the case of conventional heat developable diazotype copying materials. Further, though it has no direct bearing on the component of the light-sensitive layer, a small amount of alkali metal or alkaline earth metal salt of an organic acid such as sodium citrate, calcium citrate, magnesium citrate, sodium tartrate, calcium tartarate, calcium gluconate, etc. may be employed as a assistant dissolving agent to accelerate dissolution of the foregoing coupler in preparing a solution for use in forming the light-sensitive layer.

By applying an aqueous solution comprising the above-mentioned components dissolved therein onto one surface of a support such as paper, an acetate film, a polyester film, a synthetic paper, etc. and drying thereafter, the intended copying material can be obtained. The thus obtained heat developable diazotype copying material of the present invention is characterized not only by the production of a distinct black-color image when employed for actual copying but also by the fact that the light-sensitive layer has a satisfactory heat-resisting property. In other words, the decomposition temperatures of diazonium compounds expressed by the general Formula I or I' are comparatively higher than those of conventional diazonium compounds and are in the range of from 150° to 200° C. Accordingly, in case of a copying material employing the compounds of this invention, the decomposition loss of the diazonium compound at the time of heat development is relatively small and a highly concentrated color development can be obtained. That is, since the copying material of the present invention employs a specifically selected diazonium compound as set forth above, even if the coupling is effected at a temperature in the range of from 150° to 200° C., there will occur no loss of the diazonium compound due to heating, and a highly concentrated color development can be expected. Moreover, the copied image formed by the copying material of the present invention, that is, the dye produced thereby has excellent interceptive property for ultraviolet rays. Therefore, it has the advantage of being also applicable as the copying material for a second original for use in a diazotype copying material. Further, since the present copying material contains no alkali-producing agent in the light-sensitive layer, the preservability of the copying material per se is superb, and at the same time, it has the advantage of minimizing the discoloration of the copied image formed thereon.

#### DESCRIPTION OF THE PREFERRED EMBODIMENTS

The effect of the present invention will be further elucidated in the following comparative examples of copying materials provided with a light-sensitive layer containing just one kind of diazonium compound together with coupler expressed by the foregoing general formula and examples embodying the present invention wherein the copying material is provided with a light-sensitive layer containing at least two kinds of diazonium compounds together with said coupler.

#### COMPARATIVE EXAMPLE 1

|                                |     |     |
|--------------------------------|-----|-----|
| Water                          | ml. | 100 |
| Phloroglucinol-carboxylic acid | g.  | 3   |
| Sodium citrate                 | g.  | 2   |
| 5 Citric acid                  | g.  | 1   |
| Thiourea                       | g.  | 3   |
| Caffeine                       | g.  | 5   |
| (1)                            | g.  | 0.5 |
| Saponin                        | g.  | 0.1 |

<sup>1</sup> Formula:



15

An aqueous solution comprising the foregoing components was applied onto the surface of a support consisting of paper precoated with silica, starch, polyvinyl acetate emulsion, etc. and dried at a temperature in the range of from 100° to 120° C. After superposing the original thereon, the thus treated support was exposed by means of a mercury lamp or a fluorescent lamp in conventional method and subsequently developed by heating at 170° C. for 5 seconds. As a result, there was obtained a distinct yellow-color image formed on a white background.

#### COMPARATIVE EXAMPLE 2

|                                         |     |     |
|-----------------------------------------|-----|-----|
| Water                                   | ml. | 100 |
| 30 $\gamma$ -resorcinol-carboxylic acid | g.  | 2   |
| Sodium tartrate                         | g.  | 1   |
| Tartaric acid                           | g.  | 1   |
| Caffeine                                | g.  | 5   |
| Thiourea                                | g.  | 3   |
| 35 (1)                                  | g.  | 0.5 |
| Saponin                                 | g.  | 0.1 |

<sup>1</sup> Formula:



An aqueous solution comprising the foregoing components was treated in the same manner as in Comparative Example 1, and by treating the resultant copying material in the same way as in Comparative Example 1, coupling was effected. As a result, there was obtained a yellow-color image formed on a white background.

#### COMPARATIVE EXAMPLE 3

The below-mentioned aqueous solution (A) and aqueous solution (B) were respectively treated in the same manner as in Comparative Example 1, and subsequently by treating the resultant two kinds of copying materials in the same way as in Comparative Example 1, heat development was effected. As a result, there was obtained a yellow-color image formed on a white background in both cases.

##### Aqueous solution (A)

|                                         |     |     |
|-----------------------------------------|-----|-----|
| Components:                             |     |     |
| Water                                   | ml. | 100 |
| 55 $\gamma$ -resorcinol-carboxylic acid | g.  | 3   |
| Sodium citrate                          | g.  | 2   |
| Tartaric acid                           | g.  | 1   |
| Thiourea                                | g.  | 4   |
| Caffeine                                | g.  | 5   |
| (1)                                     | g.  | 0.5 |
| Saponin                                 | g.  | 0.1 |

<sup>1</sup> Formula:



75

7  
Aqueous solution (B)

|                                    |         |
|------------------------------------|---------|
| Components:                        |         |
| Water                              | ml. 100 |
| 3-bromo-resorcinol-carboxylic acid | g. 2    |
| Sodium acetate                     | g. 1    |
| Citric acid                        | g. 1    |
| Caffeine                           | g. 5    |
| (1)                                | g. 0.5  |
| Saponin                            | g. 0.1  |

<sup>1</sup> Formula:

## EXAMPLE 1

|                                      |         |
|--------------------------------------|---------|
| Water                                | ml. 100 |
| $\gamma$ -resorcinol-carboxylic acid | g. 3    |
| Calcium citrate                      | g. 2    |
| Citric acid                          | g. 1    |
| Thiourea                             | g. 1    |
| Caffeine                             | g. 5    |
| Guanidine sulfate                    | g. 2    |
| (1)                                  | g. 0.3  |
| (2)                                  | g. 0.5  |
| Saponin                              | g. 0.1  |

<sup>1</sup> Formula:<sup>2</sup> Formula:

An aqueous solution comprising the foregoing components was treated in the same manner as in Comparative Example 1, whereby a heat developable diazotype copying material was prepared. Subsequently, the thus prepared copying material was exposed and developed in the same way as in Comparative Example 1, and, as a result, there was obtained a distinct black-color image formed on a white background. In those cases where resorcinol-carboxylic acid employed for the foregoing aqueous solution was replaced by a member selected from the Group-A consisting of couplers expressed by the below-mentioned structural formulas, the effect was the same as in the present example.

## Group A



## EXAMPLE 2

|                                     |         |
|-------------------------------------|---------|
| Water                               | ml. 100 |
| 3-chloro-resorcinol-carboxylic acid | g. 4    |
| Sodium citrate                      | g. 4    |
| Citric acid                         | g. 1    |
| Thiourea                            | g. 2    |
| Theophylline                        | g. 7    |

8  
EXAMPLE 2—Continued

|                   |        |
|-------------------|--------|
| Guanidine sulfate | g. 3   |
| (1)               | g. 0.3 |
| (2)               | g. 0.7 |
| Saponin           | g. 0.1 |

<sup>1</sup> Formula:<sup>2</sup> Formula:

An aqueous solution comprising the foregoing components was treated in the same manner as in Example 1, whereby a heat developable diazotype copying material was prepared. As a result of employing this copying material for actual copying, there was obtained a distinct black-color image formed on a white background. In those cases where 3-chloro-resorcinol-carboxylic acid employed for the foregoing aqueous solution was replaced by a member selected from the Group-A consisting of couplers as described in Example 1, the effect was the same as in the present example.

## EXAMPLE 3

## Aqueous solution (a)

|                 |         |
|-----------------|---------|
| Components:     |         |
| Water           | ml. 100 |
| (1)             | g. 2.0  |
| Calcium citrate | g. 1.0  |
| Saponin         | g. 0.1  |

<sup>1</sup> Formula:

## Aqueous solution (b)

|                 |         |
|-----------------|---------|
| Components:     |         |
| Water           | ml. 100 |
| (1)             | g. 0.5  |
| (2)             | g. 0.5  |
| Citric acid     | g. 1.0  |
| Calcium citrate | g. 2.0  |
| Thiourea        | g. 5.0  |
| Pentaerythritol | g. 5.0  |
| Saponin         | g. 0.1  |

<sup>1</sup> Formula:<sup>2</sup> Formula:

Subsequent to applying the foregoing aqueous solution (a) onto a support consisting of paper pre-coated in the same manner as in Comparative Example 1, and drying, the coated surface was further coated with the foregoing aqueous solution (b) and dried again, whereby a heat developable diazotype copying material was prepared. The image-forming property and the color of image of this copying material proved equal to that of Example 1. In those cases where the coupler employed for the foregoing aqueous solution (a) was replaced by a member selected from the below-mentioned Group-B of couplers, the effect was the same as in the present example.

9



EXAMPLE 4  
Aqueous solution (a)

### Components:

|                                                    |    |     |
|----------------------------------------------------|----|-----|
| Water                                              | ml | 100 |
| 3,5-dichloro- $\gamma$ -resorcinol-carboxylic acid | g  | 3   |
| Calcium citrate                                    | g  | 1.5 |
| Saponin                                            | g  | 0.1 |

### Aqueous solution (b)

### Components:

|                   |    |     |
|-------------------|----|-----|
| Water             | ml | 100 |
| (1)               | g  | 0.5 |
| (2)               | g  | 0.7 |
| Citric acid       | g  | 1.0 |
| Calcium gluconate | g  | 2.0 |
| Thiourea          | g  | 5.0 |
| Pentaerythritol   | g  | 5.0 |
| Saponin           | g  | 0.1 |

### 1 Formula :



## <sup>2</sup> Formula:



The above-mentioned aqueous solution (a) and aqueous solution (b) were respectively treated in the same manner as in Example 3, whereby a heat developable diazotype copying material was prepared. As a result of employing the thus prepared copying material for actual copying, there was obtained a distinct black-color image formed on a white background. In those cases where 70 75

10

3,5-dichloro- $\gamma$ -resorcinol-carboxylic acid employed for the foregoing aqueous solution (a) was replaced by a member belonging to the Group-B of couplers described in Example 3, the effect was the same as in the present example.

**EXAMPLE 5**

### Aqueous solution (a)

## Components:

|    |                   |    |     |
|----|-------------------|----|-----|
| 10 | Water             | ml | 100 |
|    | (1)               | g  | 3.0 |
|    | Magnesium citrate | g  | 1.0 |
|    | Saponin           | g  | 0.1 |

### **<sup>1</sup> Formula :**



### Aqueous solution (b)

### Components:

|    |                   |     |     |
|----|-------------------|-----|-----|
| 25 | Water             | ml. | 100 |
|    | (1)               | g.  | 0.5 |
|    | (2)               | g.  | 0.5 |
|    | Citric acid       | g.  | 1.0 |
|    | Thiourea          | g.  | 3.0 |
| 30 | Guanidine sulfate | g.  | 1.0 |
|    | Saponin           | g.  | 0.1 |

### 2 Formula :



The above-mentioned aqueous solution (a) and aqueous solution (b) were respectively treated in the same manner as in Example 3, whereby a heat developable diazotype copying material was prepared. And, as a result of exposing and developing the thus prepared copying material in the same manner as in Example 1, there was obtained a black-color image formed on a white background.

Meanwhile, in case where the coupler employed for the foregoing aqueous solution (a) was replaced by a member of the below-mentioned Group-C of couplers, the effect was the same as in the present example.

### Group C



## 11

## EXAMPLE 6

## Aqueous solution (a)

## Components:

|                                                 |    |     |
|-------------------------------------------------|----|-----|
| Water                                           | ml | 100 |
| 4-methoxy- $\gamma$ -resorcinol-carboxylic acid | g  | 3.0 |
| Magnesium citrate                               | g  | 1.0 |
| Saponin                                         | g  | 0.1 |

## Aqueous solution (b)

## Components:

|                   |    |     |
|-------------------|----|-----|
| Water             | ml | 100 |
| (1)               | g  | 0.5 |
| (2)               | g  | 0.5 |
| Citric acid       | g  | 1.0 |
| Thiourea          | g  | 3.0 |
| Guanidine sulfate | g  | 1.0 |
| Saponin           | g  | 0.1 |

<sup>1</sup> Formula:<sup>2</sup> Formula:

The above-mentioned aqueous solution (a) and aqueous solution (b) were respectively treated in the same manner as in Example 3, whereby a heat developable diazotype copying material was prepared. And, as a result of employing the thus prepared copying material for actual copying, there was obtained a distinct black-color image formed on a white background.

In those cases where 4-methoxy- $\gamma$ -resorcinol-carboxylic acid employed for the foregoing aqueous solution (a) was replaced by a member of the Group-C of couplers described in Example 5, the effect was the same as in the present example.

## EXAMPLE 7

## Aqueous solution (a)

## Components:

|                |    |     |
|----------------|----|-----|
| Water          | ml | 100 |
| (1)            | g  | 5.0 |
| Sodium citrate | g  | 1.0 |
| Saponin        | g  | 0.1 |

<sup>1</sup> Formula:

## Aqueous solution (b)

## Components:

|                 |    |     |
|-----------------|----|-----|
| Water           | ml | 100 |
| (1)             | g  | 1.5 |
| (2)             | g  | 0.5 |
| Tartaric acid   | g  | 1.0 |
| Thiourea        | g  | 3.0 |
| Pentaerythritol | g  | 5.0 |
| Ethylene glycol | g  | 5.0 |
| Saponin         | g  | 0.1 |

<sup>1</sup> Formula:<sup>2</sup> Formula:

## 12

By means of applying the above-mentioned aqueous solution (a) and aqueous solution (b) onto the tracing paper through the same operation as in Example 3 and drying, a heat developable diazotype copying material was prepared. The image-forming property of the thus prepared copying material proved equal to those copying materials in the above Examples 3 through 6. Moreover, the copied image produced by this copying material proved suitable for use as a second original. In those cases where the coupler employed for the foregoing aqueous solution (a) was replaced by a member of the below-mentioned Group-D of couplers, the effect was the same as in the present example.

## Group D



## EXAMPLE 8

## Aqueous solution (a)

## Components:

|                                                        |    |     |
|--------------------------------------------------------|----|-----|
| Water                                                  | ml | 100 |
| 3 - ethyl - 5 - bromo - phloroglucinol carboxylic acid | g  | 5.0 |
| Sodium tartrate                                        | g  | 1.0 |
| Saponin                                                | g  | 0.1 |

## Aqueous solution (b)

## Components:

|                  |    |     |
|------------------|----|-----|
| Water            | ml | 100 |
| (1)              | g  | 1.5 |
| (2)              | g  | 0.5 |
| Tartaric acid    | g  | 1.0 |
| Thiourea         | g  | 3.0 |
| Pentaerythritol  | g  | 5.0 |
| Propylene glycol | g  | 5.0 |
| Saponin          | g  | 0.1 |

<sup>1</sup> Formula:<sup>2</sup> Formula:

The above-mentioned aqueous solution (a) and aqueous solution (b) were respectively treated in the same

manner as in Example 3 by using tracing paper as a support, whereby a heat developable diazotype copying material was prepared. And, as a result of employing the thus prepared copying material for actual copying, there was obtained a distinct black-color image formed on a white ground. In those cases where 3,5-dichloro- $\gamma$ -resorcinol-carboxylic acid employed for the foregoing aqueous solution (a) was replaced by a member of the Group-D of couplers described in Example 7, the effect was the same as in the present example. It was recognized that the copies obtained from the copying materials of the present examples are effectively applicable for the second originals.

The total molar quantity of diazonium compounds in the compositions of this invention is normally from about 0.2 to 1, based on the molar quantity of coupling compound, and the ratio of blue or purple color-producing diazonium compound to yellow color-producing diazonium compound is in the range of from about 0.2 to 2.0 mols per 1 mol of yellow color-producing diazonium compound.

What we claim is:

1. A black line heat developable diazotype copying material comprising a support and a light-sensitive layer formed onto one surface of said support wherein said layer contains:

(A) As the only coupler present a coupler selected from the group consisting of compounds having the general formula



wherein

R<sub>1</sub> and R<sub>3</sub> each is a radical selected from the group consisting of hydrogen, alkyl radicals having 1 to 6 carbon atoms, benzyl, bromine, chlorine, iodine, acetyl, and  $\omega$ -carboxyalkyl radicals having 1 to 4 carbon atoms; and

R<sub>2</sub> is a radical selected from the group consisting of hydrogen, hydroxyl radical, alkyl radical having 1 to 2 carbon atoms, alkyl-sulfonyloxy (—O—SO<sub>2</sub>-alkyl) radicals in which the alkyl group has 1 to 4 carbon atoms, carboalkoxyoxy



radicals in which the alkyl group has 1 to 4 carbon atoms, arylacyoxy



radicals having 7 to 9 carbon atoms, alkylacyloxy



radicals having 2 to 12 carbon atoms,  $\omega$ -hydroxyalkyl radicals having 1 to 3 carbon atoms,  $\omega$ -hydroxyalkyloxy radicals having 1 to 3 carbon atoms and alkoxy radicals having 1 to 4 carbon atoms;

(B) at least one diazonium compound selected from the group consisting of compounds expressed by the general Formula I



wherein

Y is a member selected from the group consisting of



(wherein R' represents a radical selected from the group consisting of hydrogen, alkyl radicals having 1 to 4 carbon atoms, hydroxyethyl radical, hydroxypropyl radical and acetyl radical); and

X is a member selected from the group consisting of —Cl<sub>1</sub>/2ZnCl<sub>2</sub>, —Cl<sub>1</sub>/2CdCl<sub>2</sub>, —Cl<sub>1</sub>/2SnCl<sub>4</sub>, —BF<sub>4</sub> and —SO<sub>3</sub>H; and general Formula I'



wherein

R'' is a radical selected from the group consisting of hydrogen, cyclohexyl radical, alkyl radicals having 1 to 4 carbon atoms, hydroxyalkyl radicals having 2 to 4 carbon atoms, cyano radical and aralkyl radicals having 7 to 11 carbon atoms;

R''' is a radical selected from the group consisting of alkyl radicals having 1 to 4 carbon atoms, aralkyl radicals having 7 to 11 carbon atoms, cyclohexyl radical, hydroxyalkyl radicals having 2 to 4 carbon atoms and benzoyl radical; and

X' is the radical identical with that of said X expressed in the general Formula I; and

(C) at least one diazonium compound selected from the group consisting of compounds having the general Formula II



wherein

R''' and R'''' each is a radical selected from the group consisting of alkyl radicals having 1 to 4 carbon atoms, hydroxyethyl radical, hydroxypropyl radical and benzyl radical; and

X'' is the radical identical with that of said X expressed in the general Formula I; and general Formula III



wherein

X''' and Y' are the radicals identical with that of said X and said Y, respectively, expressed in the general Formula I; and

R<sub>IV</sub> and R<sub>V</sub> each is a radical selected from the group consisting of alkoxy radicals having 1 to 4 carbon atoms, halogens and hydrogen; and general Formula IV



wherein

R<sub>VI</sub> and R<sub>VII</sub> each is a radical selected from the

15

group consisting of alkoxy radicals having 1 to 4 carbon atoms, halogens and hydrogen; R<sub>11111</sub> is a radical selected from the group consisting of hydrogen and alkyl radicals having 1 to 3 carbon atoms; and X''' is the radical identical with that of said X expressed in the general Formula I.

2. A diazotype copying material according to claim 1, wherein said light-sensitive layer further contains an organic acid, thiourea, and a member selected from the group consisting of guanidine sulfate, pentaerythritol, O-methyl-isothiourea and guanylurea.

3. A diazotype copying material according to claim 1, wherein said light-sensitive layer further contains a small amount of a salt selected from the group consisting of sodium citrate, calcium citrate, magnesium citrate, sodium tartrate, calcium tartrate and calcium gluconate.

4. A heat developable diazotype copying material of claim 1 wherein the coupler is a compound of the group



5. A heat developable diazotype copying material of claim 1 wherein the coupler is



6. A heat developable diazotype copying material of claim 1 wherein the coupler is



7. A heat developable diazotype copying material of claim 1 wherein the coupler is



8. A heat developable diazotype copying material of claim 1 wherein the coupler is



9. A heat developable diazotype copying material of claim 1 wherein the coupler is



10. A heat developable diazotype copying material

16

of claim 1 wherein the coupler is a compound of the group



11. A heat developable diazotype copying material of claim 1 wherein the coupler is



12. A heat developable diazotype copying material of claim 1 wherein the coupler is



13. A heat developable diazotype copying material of claim 1 wherein the coupler is



14. A heat developable diazotype copying material of claim 1 wherein the coupler is



15. A heat developable diazotype copying material of claim 1 wherein the coupler is



16. A heat developable diazotype copying material of claim 1 wherein the coupler is a compound of the group



17



17. A heat developable diazotype copying material of claim 1 wherein the coupler is



18. A heat developable diazotype copying material of claim 1 wherein the coupler is



19. A heat developable diazotype copying material of claim 1 wherein the coupler is



20. A heat developable diazotype copying material of claim 1 wherein the coupler is



21. A heat developable diazotype copying material of claim 1 wherein the coupler is



22. A heat developable diazotype copying material of claim 1 wherein the coupler is a compound of the group



18

23. A heat developable diazotype copying material of claim 1 wherein the coupler is



24. A heat developable diazotype copying material of claim 1 wherein the coupler is



25. A heat developable diazotype copying material of claim 1 wherein the coupler is



26. A heat developable diazotype copying material of claim 1 wherein the coupler is



27. A heat developable diazotype copying material of claim 1 wherein the coupler is



#### References Cited

##### UNITED STATES PATENTS

|    |           |         |                   |       |           |
|----|-----------|---------|-------------------|-------|-----------|
| 55 | 2,537,919 | 1/1957  | Slifkin           | ----- | 96-91     |
|    | 2,776,888 | 1/1957  | Pop               | ----- | 96-91     |
|    | 2,793,118 | 5/1957  | Sanders et al.    | ----- | 96-91     |
|    | 3,113,025 | 12/1963 | Bialczak          | ----- | 96-91     |
|    | 3,164,469 | 1/1965  | Behmenburg et al. | ----- | 96-49     |
|    | 3,248,220 | 4/1966  | Van Rhijn         | ----- | 96-91     |
|    | 3,331,690 | 7/1967  | Pope et al.       | ----- | 96-49     |
|    | 3,331,689 | 7/1967  | Sosnovsky et al.  | ----- | 96-49     |
|    | 3,331,869 | 7/1967  | Krueger           | ----- | 96-91 X   |
|    | 3,410,688 | 11/1968 | Welch             | ----- | 96-49 X   |
|    | 3,353,984 | 11/1967 | Landaou           | ----- | 96-91 X   |
|    | 3,565,629 | 2/1971  | Usbeck et al.     | ----- | 96-91 R   |
|    | 3,427,162 | 2/1969  | Halperin          | ----- | 96-91 R X |
|    | 3,619,191 | 11/1971 | Desjarlais        | ----- | 96-91 R X |
|    | 3,625,693 | 12/1971 | Iwaka             | ----- | 96-91 R X |

##### FOREIGN PATENTS

|           |        |               |       |       |
|-----------|--------|---------------|-------|-------|
| 1,078,912 | 8/1967 | Great Britain | ----- | 96-91 |
| 6803228   | 3/1967 | Netherlands   | ----- | 96-91 |

(Other references on following page)

**19**

## OTHER REFERENCES

Benbrook, C. H.: "The Diazotype Process," received June 1954, pp. 8 and 9.

Derwent Japanese Pat. Reports, vol. 7, No. 7, p. 6 of Section 3, March 1968 (Japanese Pat. 4127/68-Ricoh, February 1968).

**20**

Chemical Abstracts, vol. 72, Feb. 23, 1970, 37,753k.  
Chemical Abstracts, vol. 72, May 4, 1970, 95, 320c.

CHARLES L. BOWERS, JR., Primary Examiner

U.S. Cl. X.R.

96-49

Docket 8332

**UNITED STATES PATENT OFFICE**  
**CERTIFICATE OF CORRECTION**

Patent No. 3,695,885 Dated October 3, 1972

Inventor(s) Shoji Maruyama, et al

It is certified that error appears in the above-identified patent and that said Letters Patent are hereby corrected as shown below:

Column 1, line 4, change "Maryama" to read -- Maruyama --;

Column 1, line 7, after "Japan" insert --, Assignor to  
Ricoh Co. Limited, Tokyo, Japan --.

Signed and sealed this 3rd day of April 1973.

(SEAL)

Attest:

EDWARD M. FLETCHER, JR.  
Attesting Officer

ROBERT GOTTSCHALK  
Commissioner of Patents